

April 16, 1974

J. C. BOLGER ET AL  
PRODUCTION OF BLANKS USED IN THE ELECTRODEPOSITION  
OF STRIPPABLE METAL COATINGS  
Filed Dec. 11, 1972

3,804,724



FIG. 1



FIG. 2



FIG. 3

1

3,804,724

## PRODUCTION OF BLANKS USED IN THE ELECTRODEPOSITION OF STRIPPABLE METAL COATINGS

Justin C. Bolger, Dover, and Henry E. Molvar, Jr., Billerica, Mass., assignors to Canadian Copper Refiners Limited, Province of Quebec, Canada

Filed Dec. 11, 1972, Ser. No. 313,839

Inc. Cl. C23b 7/08; B01k 1/00; C09j 5/02

U.S. Cl. 204—12

23 Claims 10

### ABSTRACT OF THE DISCLOSURE

Considerably improved metal blanks are produced when edge strips made of non-conductive synthetic plastic material are bonded to the edges of such blanks using an adhesive composition based on liquid bis-phenol A type epoxy resin and dicyandiamide curing agent. Such blanks are used in the electrodeposition of strippable metal coatings such as copper cathode starting sheets.

This invention relates broadly to the electrodeposition of metals. More particularly, the invention relates to electrodeposition of strippable metal coatings, such as copper cathode starting sheets, on suitable metal blanks. The invention also covers the production of considerably improved metal blanks for the purposes mentioned above, which blanks comprise edge strips of non-conductive synthetic plastic material bonded onto at least the side edges thereof by means of an appropriate adhesive composition.

It is well known in the art of electrorefining to produce starting sheets by electrodepositing onto a blank a thin, smooth and coherent metal coating or sheet which is then stripped from the blank and used as the cathode starting sheet in the electrorefining process.

With the advent of automatic stripping machines, it has become very important to achieve a relatively easy removal of the starting sheets from the blank and several parting agents have recently been developed to facilitate this operation. One such parting agent is described in U.S. Pat. No. 3,523,873 of Aug. 11, 1970, by E. M. Elkin and consists of an aqueous emulsion comprising 2–20% by weight of a polar, saturated, substantially water-insoluble, aliphatic organic compound selected from the group consisting of fatty acids, fatty alcohols and ester and glyceride derivatives thereof and a minor amount in the range of 0.05–1% by weight of a sulfur containing material.

Although such parting agents may produce the desired result of facilitating the stripping of the electrodeposited metal sheets, they do not solve the problem of metal separation at the edges of the blanks. Indeed, during electrodeposition of the starting sheets, the metal is deposited on all exposed surfaces of the blank, including the edges, and unless special precautions are taken, the starting sheets will be bridged together by the electrodeposited metal on the edges, thereby rendering the stripping operation generally and the edge separation in particular rather difficult. To partially obviate this difficulty, slotted edge strips of non-conductive plastic material have been mounted onto the side edges of the blank and held thereon by friction. This, however, is not a very satisfactory solution, because the frictional hold is usually insufficient

2

ly tight and the electrolyte tends to penetrate between the plastic strip and the metal blank with resulting growth of metal on the edges and deformation or destruction of the plastic edge strip.

Suggestions have also been made to glue or bond the plastic edge strips to the metal blanks by means of a suitable adhesive, however, the extremely unfavorable and corrosive conditions of the hot acidic electrolytic bath lead to rapid degradation of most adhesives and the bond or weld produced by such adhesives usually fails within a few days or at the most within a few weeks. Such adhesives, therefore, do not solve the problem because it is impractical and uneconomic to replace the plastic edge strips on the metal blanks every few weeks or so, as this involves a time consuming, usually manual and therefore expensive procedure during which the blank edges and the plastic strips must be thoroughly cleaned and in some instances the plastic strips must be etched, then the adhesive must be properly applied on the blank edges as well as on the plastic strips, then the strips must be properly applied onto the edges, then the excess adhesive must be removed, then the starting sheets with the plastic strips thereon must be cured, and finally they must be inspected to make sure that everything is satisfactory.

It is obvious that in a refinery where some 5,000 to 8,000 such blanks may be continuously used to produce starting sheets, if such procedure is repeated too often, it will not be economical. Also, procedure involving additional steps or materials would again be disadvantageous and impractical.

The applicants have therefore undertaken a thorough research program to find an adhesive composition which can be applied without any special difficulty, which will satisfactorily bond or weld the plastic edge strips to the metal blanks and which will withstand the extremely unfavorable conditions of the hot acidic electrolytic bath as well as repeated stripplings of the metal coatings deposited on the blank for a period of at least one year and preferably longer, before the plastic edges need to be replaced.

It is generally known that in hot and humid conditions, it is particularly difficult to achieve a good bond between plastic materials and strongly alkaline metals, such as copper and zinc, and the applicant's research program was therefore carried out with particular emphasis on these metals, although other metals such as steel, aluminum and the like which are generally easier to bond, were also included therein.

50 A good number of adhesives which were reasonably expected to succeed have been tested. Among these were:

(1) An amine cured liquid epoxy adhesive having approximately the following composition:

|                 |             |     |
|-----------------|-------------|-----|
| Epon 828        | parts       | 100 |
| DEAPA           | do          | 6.5 |
| Silica filler   | do          | 100 |
| Cure time/temp. | hr./250° F. |     |

(2) Solvent based vinyl phenolic adhesive known under the trademark "Bloomingdale FM-47":

Cure time/temp. 1 hr. 350° F.

(3) Vinyl phenolic film adhesive known under the trademark "Bloomingdale FM-238":

65 Cure time/temp. hr./350° F. 1



invention, regular refinery copper blanks 10 were used. The upper portion of such blanks is provided with projections 11, 12 and 13 which are riveted by rivets 14 to a suspension bar 15 which supports the blank 10 when it is immersed in the electrolyte solution where starting sheets of about  $\frac{1}{16}$ " of pure copper are electrodeposited thereon.

In accordance with the present invention, the blanks 10 are provided with plastic edge strips 16 which are bonded to the edges 17 of these blanks 10 with an adhesive consisting essentially of a liquid bis-phenol A type epoxy resin combined with an effective amount of dicyandiamide curing agent. As already mentioned above, the adhesive may also comprise other constituents such as an accelerator or promoter, a flexibilizing agent and a thickener or a filler.

Two preferred but not limitative compositions of such adhesive are as follows:

(A)

|                            | Parts by weight |
|----------------------------|-----------------|
| Epon 828                   | 50              |
| Epon 872                   | 50              |
| Pulverized dicyandiamide   | 10              |
| "Cab-O-Sil"                | 2               |
| 2-ethyl-4-methyl imidazole | 0.4             |

(B)

|                       | Parts by weight |
|-----------------------|-----------------|
| Epon 828              | 100             |
| CTBN                  | 10              |
| Dicyandiamide         | 10              |
| "Cab-O-Sil"           | 3               |
| Benzyl dimethyl amine | 0.4             |

Such adhesives can be prepared in ready to use form, e.g. in the form of a paste which is stored in suitable sealed cartridges or the like. They can also be prepared in the form of premixed powder by substituting a solid bis-phenol A-type epoxy resin for the above liquid resin, to which an organic solvent such as methyl ethyl ketone may be added to achieve desired consistency. One such particularly suitable paste adhesive is known under the trademark "Uniset" A-161 of Amicon Corporation.

For copper blanks and PVC edge strips the following bonding procedure can be employed:

(1) The PVC edge strips are soaked in hot water at about 150° F. for one hour in order to pre-relax the same.

(2) The PVC edge strips are washed with a soap-water solution.

(3) The edges of the blanks are washed with soap-water solution using a bristle brush or a steel rougher, then rinsed with water, distilled water and acetone.

(4) A layer of "Uniset" A-161 adhesive is applied onto the edges of the blanks 10 and within grooves 18 of PVC edge strips 16 and allowed to set for 10-15 minutes.

(5) The edge strips are hammered onto the edges using a wooden hammer.

(6) The excess adhesive is removed from the edges.

(7) The blanks with the edge strips thereon are allowed to cure for 24 hours at room temperature or for 4 hours at 220° F.

(8) The blanks with the PVC strips bonded thereto are inspected before using them for electrodeposition of copper starting sheets.

Obviously, there may be many variations in the above procedure, however, one must ensure that the edges of the blanks and the inside grooved surfaces of the plastic strip are thoroughly cleaned and dried before applying the adhesive thereonto.

Also, although in the above procedure, edge strips made of rubberized PVC have been used, other non conducting synthetic resin materials can be employed provided they are sufficiently strong and flexible to be ap-

plied onto the edges and to withstand the conditions of electrolytic process and of successive stripping operations without cracking or degradation. For example, polyethylene edge strips have been tried and found satisfactory. However, in the case of polyethylene strips, they must be acid etched prior to bonding. An example of such acid etching procedure is as follows:

(1) The edge strips are completely immersed in a fresh solution consisting of five parts sodium dichromate, 10 eight parts tap water and one hundred parts of 95-98% sulfuric acid. The temperature of the etching bath is maintained at 60-70° C. The time of immersion is about 5 minutes.

(2) The plastic strips are then removed from the 15 etching bath and thoroughly rinsed with tap water.

(3) The strips are then dried with acetone.

There are many other etching procedures known for polyethylene and they can be adopted instead of the one described above. The man of the art should have no difficulty in finding and using a procedure that fits him best.

It is interesting to note that the bond formed between the copper blank and the polyethylene strip was so strong as to tear the polyethylene when the joint was pulled apart. Also, polyethylene edge strips do not need to be soaked in hot water to pre-relax the same as this is the case with PVC.

In addition to the above, polypropylene edge strips have been tried and again found satisfactory.

The shape of the edge strips 16 used by the applicants 30 is illustrated in FIG. 2. The groove 18 provided in these strips is generally adapted to fit closely the edge 17 of the metal blank and the outside surface of the strip is preferably rounded. However, these again are not essential features of the invention and any suitable shape or 35 form of the strips can be employed.

The edge strips 16 may be secured only to the side edges 17 of the blank 10 or they may be secured to the side edges 17 and the bottom edge 19 thereof. When they are secured only to the side edges, the bottom edge 19 is 40 usually provided with an inverted V groove 20 on the bottom surface thereof as shown in FIG. 3. This V-grooved shape of the bottom edge prevents a strong bridging of electrodeposited metal at the bottom of the blank and in most cases during stripping the copper wedge formed 45 at the bottom is weak enough to enable easy separation of the two starting sheets from one another. However, if stripping is carried out by way of automatic stripping machines using, for example, suction cups to effect the 50 stripping operation, then it may be preferable to have a plastic edge strip also at the bottom edge of the blank to achieve an easier and sharper separation.

Furthermore, when the edge strips are secured only to the side edges of the blank, it has been found preferable to extend them beyond the bottom corners of the blank 55 and to seal the remaining gap, where groove 18 is empty, by filling it with a suitable thermoplastic material such as PVC. This provides an excellent seal at the corners of the blank. Moreover, if for some reason the edge strips 16 crack after being bonded to the edges 17 of blank 10, they 60 can readily be repaired by simply sealing them with a suitable thermoplastic material.

When the metal blanks have been prepared as described above with the plastic edge strips securely bonded thereto, they may be immersed in the conventional electrolytic bath solution for electrodeposition of metallic coatings thereon. In the case of copper blanks, these are suspended in the hot copper sulfate solution containing about 20% sulfuric acid and having a temperature of about 150° F. When the required copper layer of about  $\frac{1}{16}$ " has been 65 deposited on each face of the blank, the blanks are removed, cooled in air to about 80° F. and the layers are stripped and sent for preparation as cathode starting sheets. The blanks remain in the electrolytic bath about 70 24 hours and are then removed and replaced by fresh

blanks. The same blanks are therefore undergoing approximately a 48 hour immersion cycle.

Before immersion, the blanks are preferably treated with a parting agent, for example, by dipping them into an aqueous emulsion comprising 2-20% by weight of a polar, saturated, substantially water insoluble, aliphatic organic compound selected from the group consisting of fatty acids, fatty alcohols and ester and glyceride derivatives thereof and a minor amount in the range of 0.05 to 1% by weight of a sulfur containing material, as already mentioned at the beginning of this specification.

The first two copper blanks produced in accordance with the present invention have been tested on a regular industrial scale in the refinery of Canadian Copper Refiners Limited, Montreal-East, Canada, since Feb. 12, 1971 and they are still in service with any adverse effects being evident. In addition, a whole cell using 47 blanks prepared in accordance with this invention has been tested on industrial scale in the same refinery since Aug. 14, 1971 and all these blanks are still in service without showing any adverse effects or degradation of the adhesive bond. It will be readily realized that this indeed is a surprising and unobvious result and a clear advance in the art of metal deposition. It should also be noted that the starting sheets are easily stripped from such blanks and have good sharp edges at the places where separation from the plastic edge strips is effected.

Although the specific embodiment described above refers to copper banks, this invention is by no means limited thereto. Zinc blanks, for example, can be prepared in the same manner and the plastic edge strips secured to such zinc blanks will also be entirely adequate. Metals such as steel and aluminum, which are not strongly alkaline in nature, will adhere to the plastic edge strips with even greater ease than to copper and zinc and therefore will again produce entirely satisfactory results. The invention is therefore not limited to the specifically described embodiments and many modifications obvious to those familiar with the art can be made without departing from the spirit of the invention and the scope of the following claims.

We claim:

1. Method of producing improved metal blanks used for electrodepositon of strippable metal sheets onto the opposite faces thereof, which comprises bonding onto at least the side edges of said blanks, edge strips made of non-conductive synthetic plastic material, said bonding being effected with an adhesive composition based on liquid bis-phenol A type epoxy resin and dicyandiamide curing agent.

2. Method according to claim 1, wherein said adhesive composition further comprises an effective amount of a flexibilizing agent and a thickening agent for achieving a predetermined consistency and thixotropy.

3. Method according to claim 2, wherein said flexibilizing agent is a carboxyl terminated nitrile rubber.

4. Method according to claim 2, wherein said flexibilizing agent is an ester type epoxy resin and it replaces part of the bis-phenol A type epoxy resin in the composition.

5. Method according to claim 2, wherein said thickening agent consists of colloidal silica.

6. Method according to claim 2, wherein said thickening agent is selected from the group of silica and silicate fillers.

7. Method according to claim 2, wherein the flexibilizing agent is used in a proportion between about 5 and 60% by weight relative to the weight of the bis-phenol A type epoxy resin and the thickening agent is used in the proportion between about 1 and 50% by weight relative to the weight of the epoxy resin.

8. Method according to claim 1, wherein said adhesive composition further includes an accelerator to speed the reaction between the bis-phenol A type epoxy resin and the dicyandiamide curing agent.

9. Method according to claim 8, wherein said accelerator is selected from the group consisting of nitrogenous compounds and acid salts thereof.

10. Method according to claim 9, wherein said nitrogenous compounds are selected from the group consisting of tertiary amines, ureas, guanidines and imidazoles.

11. Method according to claim 8, wherein said accelerator is used in a proportion of 0.1-20% by weight with respect to the weight of the bis-phenol A type epoxy resin.

12. Method according to claim 1, wherein said blanks are copper blanks.

13. Method according to claim 1, wherein said plastic strips are made of PVC.

14. Method according to claim 1, wherein said plastic strips are made of polyethylene or polypropylene.

15. Method according to claim 1, wherein said plastic strips are bonded to the side edges and to the bottom edge of the metal blank.

16. Method according to claim 1, wherein said plastic strips are bonded only to the side edges of the metal blank and the bottom edge surface of said blank is provided with a groove in the form of an inverted V over its entire length.

17. Method according to claim 1, wherein said plastic strips are of rounded configuration and have a groove in the middle thereof adapted to be tightly fitted over the edges of the metal blank.

18. Method of producing improved copper blanks used for electrodeposition in a hot acidic electrolyte of copper starting sheets on the opposite faces thereof, which comprises bonding onto at least the side edges of said blanks, edge strips made of non conductive synthetic plastic material capable of withstanding the hot acidic electrolyte and the abuse of repeated starting sheet stripping operations, said plastic edge strips being bonded using the following procedure:

(a) the edges of the blanks and the plastic strips are thoroughly cleaned and dried;

(b) a layer of adhesive composition based on liquid bis-phenol A type epoxy resin and dicyandiamide curing agent is applied onto the edges of the blank and onto the surfaces of the plastic strips to be bonded thereto.

(c) the adhesive is allowed to set;

(d) the plastic edge strips are secured to the edges of the blank and any excess adhesive is removed; and

(e) the adhesive is allowed to cure.

19. Method according to claim 18, wherein the plastic edge strips are of PVC and are pre-relaxed by soaking them in hot water prior to cleaning them and applying the adhesive thereonto.

20. Method according to claim 18, wherein the plastic edge strips are of polyethylene and are acid etched prior to cleaning them and applying the adhesive thereto.

21. A method of making copper cathode starting sheets which comprises forming a copper blank comprising edge strips made of non conductive synthetic plastic material bonded onto at least the side edges thereof by means of an adhesive composition based on liquid bis-phenol A type epoxy resin and dicyandiamide curing agent, applying onto said blank a coating of a parting agent, electrodepositing substantially pure copper on the opposite faces of said blank, stripping the resulting electrodeposited copper sheets from said surfaces of the blank in the form of smooth, coherent copper sheets with sharp edges, and reusing the same blanks for successive operations on a 48 hour cycle for at least one year, before replacement of the plastic edge strips may be needed.

22. Method according to claim 21, wherein said parting agent is an aqueous emulsion comprising 2-20% by weight of a polar, saturated, substantially water-insoluble, aliphatic, organic compound selected from the group consisting of fatty acids, fatty alcohols and ester and glyceride derivatives thereof and a minor amount in

3,804,724

9

the range of 0.05-1% by weight of a sulfur-containing material.

23. Method according to claim 1, wherein said electro-deposited copper sheets are stripped off the blanks by an automatic stripping machine.

10

|             |        |            |       |         |
|-------------|--------|------------|-------|---------|
| 3,386,956   | 6/1968 | Nawakowski | ----- | 260-47  |
| 3,391,113   | 7/1968 | Lopez      | ----- | 260-47  |
| 3,530,047   | 9/1970 | Billett    | ----- | 204-12  |
| 3,556,928   | 1/1971 | Zolg       | ----- | 156-330 |
| 5 3,562,215 | 2/1971 | Moore      | ----- | 260-47  |

References Cited

UNITED STATES PATENTS

|           |        |          |       |         |
|-----------|--------|----------|-------|---------|
| 1,994,144 | 3/1935 | Merrill  | ----- | 204-281 |
| 2,343,161 | 2/1944 | Tetrault | ----- | 204-297 |

THOMAS M. TUFARIELLO, Primary Examiner

U.S. Cl. X.R.

10 156-307, 330; 204-281

UNITED STATES PATENT OFFICE  
CERTIFICATE OF CORRECTION

Patent No. 3,804,724

Dated April 16, 1974

Inventor(s) Justin C. Bolger and Henry E. Molvar, Jr.

It is certified that error appears in the above-identified patent  
and that said Letters Patent are hereby corrected as shown below:

Claim 23 should read:

-- Method according to claim 21, wherein said electro-  
deposited copper sheets are stripped off the  
blanks by an automatic stripping machine. --

Column 4, line 55, "1969" should correctly read  
-- 1968 --

Signed and sealed this 1st day of October 1974.

(SEAL)

Attest:

McCOY M. GIBSON JR.  
Attesting Officer

C. MARSHALL DANN  
Commissioner of Patents

UNITED STATES PATENT OFFICE  
CERTIFICATE OF CORRECTION

Patent No. 3,804,724 Dated April 16, 1974

Inventor(s) Justin C. Bolger and Henry E. Molvar, Jr.

It is certified that error appears in the above-identified patent  
and that said Letters Patent are hereby corrected as shown below:

Column 7, line 16, "with" should correctly  
read -- without --

line 44, (Claim 1), "electrodeposition"  
has been misspelled

Signed and sealed this 3rd day of December 1974.

(SEAL)

Attest:

McCOY M. GIBSON JR.  
Attesting Officer

C. MARSHALL DANN  
Commissioner of Patents